

1

2,781,904

**METHOD OF DEWATERING AND DRESSING  
VERY FINE-GRAINED MINERAL SUB-  
STANCES**

Wilhelm Reerink, Essen-Bredeney, Walter Müschenborn,  
Essen, and Erich Nötzold, Essen-Haarzopf, Germany

No Drawing. Application January 12, 1954,  
Serial No. 403,668

Claims priority, application Germany January 14, 1953

11 Claims. (Cl. 209—12)

The invention relates to a method of dewatering and dressing very fine-grained mineral substances, such as coal slurries, small ores and the like, namely such raw materials themselves and in particular concentrates, existing in the form of very fine grains, from a previous dressing treatment, said method not only permitting particularly simple and intensive dewatering of such substances but also being capable of combination in an advantageous manner with a dressing treatment or further dressing treatment of such substances.

The dewatering of very fine-grained mineral substances is known to give rise to extremely great difficulties both because of the small quantitative output of known apparatus and also because of the degree of dewatering obtainable with the aid of such apparatus.

Thus, for example, in the dewatering of coal flotation concentrates on filters, with the use of very fine screens or filter cloth tensions with a correspondingly low output, a reduction of the water content to at best 18—25% can be obtained.

The difficulties of dewatering are increased as the grain size of the material falls, particularly when very fine debris particles (clays) are still contained therein.

In the dewatering of crude slurries, which always contain such very fine debris particles, the output and result of the filtration are so poor that mechanical dewatering of such slurries in this manner is of doubtful success.

When centrifuges are used it is true that a considerable reduction of the water content is possible, but considerable losses of solids with the water passing through the screen linings of the centrifuges must be faced. These losses of solids increase as the wear on the screens increases and, as the latter always wear very rapidly, the losses may amount to as much as 400 g. per litre. Since such losses cannot be tolerated, the very fine slurries centrifuged through the screens must be further subjected to after-treatment by concentration or in cyclones, and then recycled to the centrifuge. Nevertheless, the very fine solids gradually accumulate in the water and must be removed by other means, namely by still more difficult filtering.

The invention renders it possible to effect very substantial dewatering of very fine-grained materials, such as slurries and flotation concentrates, in screening centrifuges, while avoiding these difficulties, and possibly at the same time to purify the concentrates still further. According to the invention this is achieved by subjecting the material, before it is charged to the screening centrifuge (basket centrifuge or thrust centrifuge), to previous treatment with substances by which the coal particles are coated with an envelope rendering them hydrophobic.

It has already been proposed to subject very fine-grained mineral substances to treatment with oil, accompanied by dispersion in water, and then to pass them to a screening centrifuge. This proposal constitutes primarily a dressing method which aims at bringing the debris constituents into the form of a suspension and then in the screening centrifuge separating into coal or concentrate

2

and debris-containing waste water, which is discharged. It entails the use of relatively large amounts of highly viscous oils and special steps in the course of the wetting of the particles, in order on the one hand to ensure that all the particles of coal are enveloped in oil, and on the other hand to prevent coal particles from passing through the screen linings with the debris water.

In contradistinction thereto, it is the main task of the present invention to dewater the material while recovering the material contained in the matter passing through the screen of the centrifuge, it being thus not necessary to pay any attention to the greatest possible avoidance of losses in the matter passing through the screen. For this reason, the pre-treatment serving to render the particles hydrophobic can be carried out with the aid of substantially smaller amounts of oils, namely oils of any type, even those of low viscosity, or other suitable reagents having the effect of rendering the particles hydrophobic, such as hydrocarbons, xanthates, and the like, while it is possible to absorb without difficulty fluctuations both in respect of the amounts and in respect of the distribution of the grain sizes and of the solid content of the slurry treated.

The particles can be rendered hydrophobic in fundamentally similar manner to that in the known method of dressing, by treating the material with a relatively small amount of substances rendering it hydrophobic, while it passes through a baffle-plate mill, or machines having a similar action, such as kneading mechanisms, high-speed agitators, or machines known as homogenising machines, if desired with simultaneous comminution, while by the addition of suitable reagents to be selected according to the conditions prevailing in the individual case, it is possible not only to improve the result of the hydrophobisation, but also to reduce the amounts of hydrophobising substances required.

The slurry treated in this manner is charged to the centrifuge basket, preferably in as highly concentrated a condition as possible, with a high solid content.

Through the preceding hydrophobisation, the passage of the very fine grains through the centrifugal screens is on the one hand avoided to a great extent, being reduced to a fraction, while on the other hand the moisture content of the centrifuged material can be reduced still further with a high output, namely in certain circumstances to values such as hitherto could not be achieved.

When the material to be dewatered is already in the form of a pure concentrate, for example one coming from a preceding flotation dressing treatment, its ash content on passing through the centrifuge is further lowered because the non-hydrophobic and generally highly dispersed debris fragments which are always still present even in pure concentrates, even if in small amounts, pass through the centrifuge screens to a considerable extent together with the water.

In the material passing through the centrifuge the hydrophobised coal or ore particles contained therein will generally spontaneously float to the surface and can be removed in the simplest manner and recharged to the centrifuge, while the residual water can be discharged.

In the case of substances which do not float of their own accord after passing through the centrifuge, as a further development of the new process the material passing through the centrifuge can be subjected to flotation treatment, either by the simple injection of air or in a subsequent flotation cell, the concentrate from which treatment is returned to the centrifuge in the same manner; in either case the method of the invention ensures practically loss-free continuous dewatering, while the content of wrongly discharged material (losses of concentrates) in the filtrate water is very low.

When the new process is applied to the treatment of

crude slurries, flotation treatment is inserted between the hydrophobising treatment carried out in the same manner as described above and the centrifugal treatment. It is then found particularly advantageous that the pretreated material, including substances which can otherwise be floated only poorly or not at all, is readily floatable in the hydrophobised condition thus attained.

In fundamental contradistinction to the earlier, previously mentioned method of dressing, however, here also the centrifugal treatment serves substantially only for dewatering, by which all the debris particles, which are of course also dispersed in the water, are likewise separated, while the separation of the major part of the debris is effected previously, namely in the flotation.

In these circumstances, in this case the hydrophobising treatment can be transferred to the flotation plant itself, i. e. be carried out together with the flotation treatment.

The effect of the latter is that the new process is merely used for the loss-free dewatering of normal flotation concentrates, i. e. follows known flotation plants instead of the otherwise necessary filter and similar dewatering plants.

The fundamental advantage of the new process from the point of view of dressing, in relation to the process previously proposed by us, is based on the fact that the very fine-grained concentrate losses contained in the filtrate water of the centrifuge are directly reconcentrated and returned to the dewatering stage, and thus cannot accumulate in the water. The highly dispersed very fine debris contained in the concentrate is separated therefrom through the centrifugal treatment and therefore cannot render difficult the dewatering process as in normal dewatering by means of filters. On repetition of the centrifugal treatment they are discharged to the waste water in the flotation cell.

A further considerable simplification of the method described is achieved if, according to a further feature of the invention, the hydrophobising treatment is transferred to the centrifuge itself, the substances to be dressed being charged directly to the centrifuge together with the oils and, if required, reagents.

The wetting of the particles is then effected through the turbulence in the admission guide mechanism or on passing through the narrow admission slots, or on the passing of the very fine particles through the screen apertures in the presence of very finely divided hydrophobising substances. The centrifuge losses are reconcentrated in the manner described above, for example by flotation, and recentrifuged.

This form of carrying out the method is, however, not applicable in all cases but only where particularly favourable conditions exist in respect of the ability of the concentrate particles to be rendered hydrophobic.

In similar manner, fine-grained concentrates from other concentration processes, such as concentrates produced by dressing on concentrating tables by means of cyclones or the like, can be dewatered.

Some examples of the new method are given below:

#### Example I

A coal flotation concentrate, which after the material charged had first been rendered hydrophobic was produced with an ash content of 12%, was charged to the screening centrifuge.

The dewatered concentrate produced in the screening centrifuge contained 6.5% of ash and 9% of water. The matter passing through the centrifuge had an ash content of 36% and was returned to the flotation treatment for redressing. The material leaving the flotation process contained 75% of ash.

#### Example II

An anthracitic fine coal of a grain size below 1 mm., which in itself is not floatable, was passed with a small percentage of fuel oil per ton, with the addition of soda

solution, through a baffle-plate mill and thereupon charged to a stirring mechanism flotation apparatus, in which pure debris containing over 80% of ash was discharged.

The concentrate of this flotation was charged to the screening centrifuge with a solid content of 450 g. per litre.

A water content of the dewatered material amounting to 11% was obtained, while the material passing through the centrifuge, which consisted of coal and very fine debris, contained 35% of ash and the slurry had a solid content of 40 g. per litre. This material leaving the centrifuge was returned to the flotation.

#### Example III

A crude ore having a sulphur content of 70 to 75% was passed with flotation oil through a baffle-plate mill and simultaneously ground and hydrophobised in the latter.

The material treated in this manner was separated in a flotation plant into a foam having a high solid content and debris and the foam was passed to a screening centrifuge, in which it was dewatered to a water content of 9%. The relatively pure matter passing through the screening centrifuge was returned to the flotation. The concentrate obtained had a sulphur content of 98.6%.

We claim:

1. A method of dewatering and dressing very fine-grained substances which comprises in combination the steps of hydrophobising said substances, continuously centrifugally screening the hydrophobised substances, separating the matter passing through the centrifugal screen into floatable particles and waste water, and returning the floating fraction to the continuous centrifugal screening.

2. A method of dewatering and dressing very fine-grained substances which comprises in combination the steps of subjecting said substances to treatment with oil-containing substances to render them hydrophobic, continuously centrifugally screening the hydrophobised substances, separating the matter passing through the centrifugal screen into floatable particles and waste water, and returning the floating fraction to the continuous centrifugal screening.

3. A method of dewatering and dressing very fine-grained substances which comprises in combination the steps of subjecting said substances to treatment with a reagent to render them hydrophobic, continuously centrifugally screening the hydrophobised substances, separating the matter passing through the centrifugal screen into floatable particles and waste water, and returning the floating fraction to the continuous centrifugal screening.

4. A method of dewatering and dressing a coal slurry which comprises in combination the steps of hydrophobising the coal particles of said slurry, continuously centrifugally screening the hydrophobised slurry, separating the matter passing through the centrifugal screen into floatable particles and waste water, and returning the floating fraction to the continuous centrifugal screening.

5. A method of dewatering and dressing very fine ores which comprises in combination the steps of hydrophobising said ores, continuously centrifugally screening the hydrophobised ores, separating the matter passing through the centrifugal screen into floatable particles and waste water, and returning the floating fraction to the continuous centrifugal screening.

6. A method of dewatering and dressing very fine-grained substances which comprises in combination the steps of hydrophobising said substances, continuously centrifugally screening the hydrophobised substances, subjecting the matter passing through the centrifugal screen to flotation treatment, and returning the concentrate from said flotation treatment to the continuous centrifugal screening.

7. A method of dewatering and dressing very fine-

grained substances which comprises in combination the steps of hydrophobising said substances, subjecting said hydrophobised substances to flotation treatment, subjecting the concentrate from said flotation treatment to continuous centrifugal screening and recycling the matter passing through the centrifugal screen to said flotation treatment.

8. A method of dewatering and dressing very fine-grained substances which comprises in combination the steps of hydrophobising said substances in a baffle plate mill, continuously centrifugally screening the hydrophobised substances, separating the matter passing through the centrifugal screen into floatable particles and waste water, and returning the floating fraction to the continuous centrifugal screening.

9. A method of dewatering and dressing very fine-grained substances which comprises in combination the steps of hydrophobising and simultaneously kneading said substances, continuously centrifugally screening the hydrophobised and kneaded substances, separating the matter passing through the centrifugal screen into floatable particles and waste water, and returning the floating fraction to the continuous centrifugal screening.

10. A method of dewatering and dressing very fine-grained substances which comprises in combination the

steps of hydrophobising and simultaneously comminuting and homogenising said substances, continuously centrifugally screening the hydrophobised comminuted and homogenised substances, separating the matter passing through the centrifugal screen into floatable particles and waste water, and returning the floating fraction to the continuous centrifugal screening.

11. A method of dewatering and dressing very fine-grained substances which comprises in combination the steps of hydrophobising said substances in flotation plant, subjecting the concentrate from said combined hydrophobising and flotation treatment to continuous centrifugal screening and recycling the matter passing through the centrifugal screen to said combined hydrophobising and flotation treatment.

References Cited in the file of this patent

UNITED STATES PATENTS

1,338,264      Thornhill \_\_\_\_\_ Apr. 27, 1920  
2,113,727      Hall et al. \_\_\_\_\_ Apr. 12, 1938

OTHER REFERENCES

Bureau of Mines Information Circular 7660, "Convertol Process of Coal-Slurry Treatment," by Thomas Fraser, April 1953. (4 pp. descr.; 3 shts. drwg.)